# EUROPEAN PATENT SPECIFICATION

(11) **EP 2 223 803 B1**
(45) Date of publication and mention of the grant of the patent: **02.11.2011**
(21) Application number: 10152343.9
(22) Date of filing: 02.02.2010
(51) Int. Cl.: B41C 1/00

(54) **Preparation of flexographic printing masters using an additive process**
Herstellung von flexografischen Druckvorlagen mittels eines Additivverfahrens
Préparation de supports d'impression flexographiques utilisant un procédé additif

(30) Priority: 26.02.2009 US 393230
(43) Date of publication of application: 01.09.2010
(73) Proprietor: Xerox Corporation, Rochester, NY 14644 (US)
(72) Inventor: Keoshkerian, Barkev, Thornhill Ontario L4J 7E8 (CA); Belelie, Jennifer L., Oakville Ontario L6N 4A5 (CA); Chopra, Naveen, Oakville Ontario L6H 5W4 (CA); Chretien, Michelle, Mississauga Ontario L5N 1J2 (CA)
(74) Representative: Grünecker, Kinkeldey, Stockmair & Schwanhäusser

(56) References cited:
- EP-A1- 1 428 666
- EP-A2- 1 449 648
- US-A1- 2004 129 158

## Description

Flexographic printing is a method of direct rotary printing that uses a resilient relief image carrier to print articles such as cartons, bags, labels, newspapers, food or candy wrappers or books. Flexographic printing has found particular application in packaging, where it has displaced rotogravure and offset lithography printing techniques in many cases. Flexographic plates can be prepared from a printing plate precursor having a layer consisting of a photo-polymerizable composition, which generally comprises an elastomeric binder, at least one monomer and a photo-initiator. Early patents on flexographic printing plates include U.S. Pat. No. 3,960,572, U.S. Pat. No. 3,951,657, U.S. Pat. No. 4,323,637 and U.S. Pat. No. 4.427,759.

Traditionally, an image to be printed is formed in a flexographic printing plate precursor material by exposing the photo-polymerizable layer of the flexographic printing plate to ultraviolet radiation with an image mask interposed between the radiation source and the printing plate precursor. The ultraviolet radiation causes polymerization to occur in the areas of the photo-polymerizable layer not shielded by the image mask. After imaging, the plates are processed with a suitable solvent to remove the photo-polymerizable composition in the unexposed areas, thereby creating a relief-based image on the printing plate. The processed plates are then mounted on a printing press, where they are used to transfer ink in the pattern formed in the printing plate to a desired printing surface.

The above process for manufacturing a flexographic printing plate was simplified by applying a layer for forming the image mask directly on the printing plate precursor. U.S. Pat. No. 6.521,390 describes the "direct laser process", wherein an IR-ablatable layer, substantially opaque to ultraviolet radiation, was laminated on the flexographic printing plate precursor and removed by an IR laser. The printing relief was produced upon exposing the image mask to ultraviolet light, and thus crosslinking photosensitive material on the printing relief. Various representations of the "direct laser process" are described in EP-A 654150, U.S. Patent No. 5.259,311 and U.S. Patent No. 6,880,461. Even though the above process for preparing the flexographic printing plate was simplified by incorporating an image mask forming layer into the printing plate precursor, the process remains complicated and time-consuming. Furthermore, the process is not environment-friendly due to a high waste production in removing the unexposed areas of the photo-polymerizable layer by the IR laser.

U.S. Pat. No. 5,511,477 discloses a method for the production of photopolymeric relief-type printing plates comprising the steps of forming a positive or negative image on a substrate by ink jet printing with a photopolymeric ink composition, optionally preheated to a temperature of about 30 to 260°C; and of subjecting the resulting printed substrate to UV radiation, thereby curing the ink composition forming the image. Suitable substrates for this method are restricted to steel, polyester and other rigid materials, limiting the possibilities for flexographic applications. Another problem is that jetted droplets of the polymeric ink are still mobile and tend to deform, thereby preventing accurate reproduction of small dots and preventing the formation of sharp edges and hence the formation of a sharp image.

U.S. Pat. No. 6,520,084 discloses a method for manufacturing a flexographic printing plate by means of multiple passes of an ink-jet unit employing two different elastomers that are deposited on a modifying surface. For jetting, the elastomers can be liquefied by heating meltable polymers to temperatures between 100 and 150°C or by dissolving them in hazardous and toxic solvents such as toluene. The requirement of high temperatures restricts not only the choice of suitable substrates, but also limits the ink-jet printer to a "solid ink-jet" device. The toluene is allowed to evaporate between every two deposited layers, creating a hostile environment.

EP-A 1428666 discloses a method for preparing a flexographic printing plate by jetting radiation curable inkjet ink on a resilient substrate. The disclosed inks do not contain any elastomers and the quality of the flexographic printing plate is inferior to conventional flexographic printing plates.

U.S. Patent No. 7.401,552 describes a method for preparing a flexographic printing plate by a) providing an ink-receiver surface; (b) jetting a curable jettable fluid on the ink-receiver surface **characterized in that** the curable jettable fluid comprises at least one photo-initiator, at least one monofunctional monomer, at least 5 wt % of a polyfunctional monomer or oligomer and at least 5 wt % of a plasticizer both based on the total weight of the curable jettable liquid, capable of realizing a layer after curing having an elongation at break of at least 5%, a storage modulus E' smaller than 200 mPa at 30 Hz and a volumetric shrinkage smaller than 10%.

US-A-2004/0129158 discloses a method of digitally building up flexographic plates, comprising the steps of:
a) providing a plate substrate and an imaging surface;
b) depositing an electrometric matrix floor onto said plate substrate;
c) curing said deposited matrix floor;
d) ink-jet imaging one layer of said imaging surface according to pre-stored digital image data;
e) UV exposing said image layer to create a gelled layer;
f) transferring said gelled layer from the imaging surface to the surface of the matrix floor on said plate substrate;
g) bonding said gelled layer with the matrix floor; and
h) repeating steps d) to g) until an image of sufficient thickness is created on said plate substrate.

EP-A-1449648 discloses a method for making a relief printing plate having ink-receptive cured areas on a receiver base, the method comprising the steps of:
(a) imaging a lithographic printing plate precursor to produce a lithographic printing plate having ink-receptive image areas and ink-repellent non-image areas, the ink-receptive image areas and ink-repellent non-image areas defining a first image;
(b) applying a first curable composition to the lithographic printing plate, wherein the first curable composition wets the ink-receptive image areas and does not wet ink-repellent non-image areas, to form a substantially uniform coating of the first curable composition on ink-receptive image areas;
(c) contacting the coating of the first curable composition to the receiver base to make an impression of the first curable composition on the receiver base; and
(d) curing the impression on the receiver base to produce a first cured layer, such that the first cured layer includes ink-receptive cured areas defining a second image corresponding to the first image.

While the quality of articles printed using flexographic plates has improved significantly as the technology has matured, physical limitations related to the process of creating a relief image in a plate remain.

There is therefore a need for a fast, simple and environmental friendly method for manufacturing a flexographic printing plate with a high image quality, and applicable to a wide range of applications, including printing on soft and easily deformable surfaces.

The above and other issues are addressed by the present application, wherein in embodiments, the application relates to a method of forming a printing master on a flexographic plate, by first melting a radiation-curable phase change ink and depositing at least one drop of the melted ink on the flexographic plate in a pattern to form a first layer of an image. After the first layer of the ink is allowed to gel on the flexographic plate, an additional layer or additional layers are formed on top of the first layer, each successive layer being gelled prior to deposition of subsequent layers, until a printing master with sufficient thickness is formed on the flexographic plate. Only after the printing master with a sufficient thickness is formed, is the built up stack of jetted layers cured.

In embodiments, described is a method of forming a printing master on a flexographic plate, the method comprising: (a) melting a radiation-curable phase change ink comprised of at least one curable monomer, at least one phase change agent, at least one photoinitiator and an optional colorant, (b) depositing multiple layers of the melted ink at desired locations on the flexographic plate to form a raised pattern, wherein each deposited layer of ink is gelled prior to the deposition of a subsequent layer on the deposited layer, until the printing master with sufficient thickness is formed on the flexographic plate, and (c) curing the ink on the flexographic plate upon the conclusion of the depositing step.

In further embodiments, described is a method of forming a printing master on a flexographic plate, the method comprising: (a) melting a radiation-curable phase change ink comprised of at least one curable monomer, at least one gellant, at least one photoinitiator and an optional colorant, (b) depositing the melted ink on the flexographic plate in a pattern to form a layer of the pattern, (c) allowing the deposited layer of the of the ink to gel on the flexographic plate, (d) depositing the melted ink on the previous deposited layer to form an additional layer, (e) allowing the deposited additional layer to gel, (f) repeating steps (d) through (e) to form further additional deposited and gelled layers, until the printing master with sufficient thickness is formed on the flexographic plate, and (g) curing the ink on the flexographic plate upon the achievement of the sufficient thickness, wherein the viscosity of the melted ink is from 0.001 to 100 Pa·s (10⁰ cP to 10⁵ cP) at a temperature of from 60°C to 100°C.

In further embodiments, described is a method of forming a printing master on a flexographic plate, the method comprising: (a) melting a radiation-curable phase change ink comprised of at least one curable monomer, at least one phase change agent, at least one photoinitiator and an optional colorant, (b) depositing the melted ink on the flexographic plate in a pattern to form a layer in the pattern, (c) allowing the deposited layer of the of the ink to gel on the flexographic plate, (d) depositing an additional layer of the melted ink on the previous deposited layer, (e) allowing the deposited additional layer to gel, (f) repeating steps (d) through (e) to form further additional deposited and gelled layers, until the printing master with an initial thickness is formed on the flexographic plate, (g) curing the ink on the flexographic plate to form an initial portion of the printing master, (h) depositing a post-initial curing layer of the melted ink on the initial portion of the printing master, (i) allowing the deposited post-initial curing deposited layer of the melted ink to gel on the flexographic plate, (j) depositing an additional post-initial curing layer of the melted ink on the previous deposited post-initial curing deposited layer, (k) allowing the deposited additional post-initial curing additional layer to gel, (1) repeating steps (j) through (k) to form further additional post-initial curing deposited and gelled layers, until the printing master with sufficient thickness is formed on the flexographic plate, and (m) curing the ink on the flexographic plate upon the achievement of the sufficient thickness.

Preferred embodiments are set forth in the subclaims.

Described herein is a method of forming a printing master on a flexographic plate, the method comprising: (a) melting a radiation-curable phase change ink. (b) depositing multiple layers of the melted ink at desired locations on the flexographic plate to form a raised pattern, wherein each deposited layer of ink is gelled prior to the deposition of a subsequent layer on the deposited layer, until the printing master with sufficient thickness is formed on the flexographic plate, and (c) curing the ink un the flexographic plate upon the conclusion of the depositing step.

Furthermore, described herein is a method of forming a printing master on a flexographic plate, the method comprising: (a) melting a radiation-curable phase change ink comprised of at least one curable monomer, at least one gellant, at least one photoinitiator and an optional colorant, (b) depositing the melted ink on the flexographic plate in a pattern to form a layer of the pattern, (c) allowing the deposited layer of the of the ink to gel on the flexographic plate, (d) depositing the melted ink on the previous deposited layer to form an additional layer, (e) allowing the deposited additional layer to gel, (f) repeating steps (d) through (e) to form further additional deposited and gelled layers, until the printing master with sufficient thickness is formed on the flexographic plate, and (g) curing the ink on the flexographic plate upon the achievement of the sufficient thickness, wherein the viscosity of the melted ink is from 0.001 to 100 Pa·s (10⁰ cp to 10⁵ cP) at a temperature of from 60°C to 100°C.

Radiation curable phase change inks generally comprise at least one curable monomer, at least phase change agent, and an optional colorant. They may further comprise at least one photoinitiator that initiates polymerization of the curable monomer. Exemplary phase change inks suitable for use include those described in U.S. Patent Nos. 7,276,614 and 7,279,587 and U.S. Patent Application Publication Nos. 2007/0120908; 2007/0120909; 2007/0120925 and 2008/0128570. The printing processes of the present disclosure take advantage of this rapid change in the viscosity to limit lateral ink spreading along the surface of the printing plate material prior to curing.

The phrase "radiation curable" herein refers to, for example, the ability of the phase change ink to be cured by radiation so that it becomes permanently fixed to the flexographic plate. All forms of curing upon exposure to a radiation source are contemplated, including light and heat sources in the presence or absence of initiators. Exemplary radiation curing routes include, for example, curing using ultraviolet (UV) light, for example having a wavelength of 200 to 400 nm, or more rarely using visible light, curing using electron beam radiation, curing using thermal curing, and appropriate combinations thereof.

The curing of the curable monomer may be a radically initiated curable monomer, cationically initiated curable monomer or a combination of a radically initiated and cationically initiated curable monomer. In embodiments, the monomer is equipped with one or more curable moieties, including, but not limited to, acrylates; methacrylates; vinyl ethers; epoxides, such as cycloaliphatic epoxides, aliphatic epoxides, and glycidyl epoxides; oxetanes; and the like. Suitable radiation, such as UV, curable monomers may include acrylated esters, acrylated polyesters, acrylated ethers, acrylated polyethers, acrylated epoxies, urethane acrylates, and pentaerythritol tetraacrylate and combinations thereof. Specific examples of suitable acrylated monomers include monoacrylates, diacrylates, and polyfunctional alkoxylated or polyalkoxylated acrylic monomers comprising one or more di- or tri-acrylates and combinations thereof.

Advantageous properties can be obtained when monomers are alkoxylated, such as ethoxylated or propoxylated, for example: propoxylated neopentyl glycol diacrylate, ethoxylated neopentyl glycol diacrylate, propoxylated hexanediol diacrylate. In embodiments, one suitable monomer is a propoxylated neopentyl glycol diacrylate, such as, for example, SR-9003 (Sartomer Co., Inc., Exton, Pa.).

The curable monomer may be present in the ink in an amount of, for from 20 to 90% by weight of the ink, such as 30 to 85% by weight of the ink, or 40 to 80% by weight of the ink.

The radiation curable phase change inks may also include a phase change agent. The inclusion of a phase change agent in some phase change inks allows the inks to "phase change" or undergo a sharp increase in viscosity over a narrow temperature range upon heating the ink to a temperature above room temperature, and harden to a gel-like consistency, which is retained as the inks are cooled further to room temperature. For example, some phase change inks which may be suitable for use in the devices and methods of the present disclosure have a viscosity which changes by a factor of 10⁴ to 10⁹ over a temperature change of only 20 to 40°C.

The phase change agent may generally be any component that is miscible with the other components of the phase change ink and promotes the increase in viscosity of the ink as it cools from the jetting temperature to the flexographic plate temperature. Examples of classes of phase change agents include gellants and waxes.

In embodiments, the inclusion of a phase change agent in the radiation curable phase change inks may result a change in viscosity of least 0.1 Pa·s 10² (centipoise (cP)). 0.1 Pa·s for example, from 0,001 to 100 Pa·s (10⁰ cP to 10⁵ cP), from 0.001 to 10 Pa·s (10⁰ to 10⁴), from 0,01 to 0,1 Pa·s (10¹ to 10²), from 0,1 to 100 Pa·s (10² cP to 10⁵ cP) and from 10 to 1000 Pa·s (10⁴ cP to 10⁶ cP) over a temperature range of, for example, in one embodiment at least 30°C, for example, from 40°C to 120°C, from 60°C to 100°C and 70°C to 95°C.

In embodiments, a gellant is used as the phase change agent. The gellant compositions disclosed herein can act as an organic gellant in the ink to the viscosity of the ink within a desired temperature range. In particular, the gellant may form a semi-solid gel in the ink vehicle at temperatures below the specific temperature at which the ink is jetted.

Any suitable gellant, may be used for the ink vehicles disclosed herein. Specifically, the gellant can be selected from materials disclosed in U.S. Pat. No. 7,279,587 and U.S. Pat. No. 7,276,614 such as a compound of the formula

R₃-X-CO-R₂-CO-NH-R₁-NH-CO-R₂'-CO-X'-R₃',

wherein: R₁ is selected from the group consisting of an alkylene group, an arylene group, an arylalkylene group and an alkylarylene group; R₂ and R₂' are selected from the group consisting of an alkylene group, an arylene group, an arylalkylene group and an alkylarylene group; R₃ and R₃' are selected from the group consisting of a photoinitiating group, an alkyl group, an aryl group, an arylalkyl group and an alkylaryl group; and X and X' is an oxygen atom or a group of the formula--NR₄--.

The alkylene group for R₁ is defined as a divalent aliphatic group or alkyl group, including linear and branched, saturated and unsaturated, cyclic and acyclic, and substituted and unsubstituted alkylene groups, and wherein heteroatoms, such as oxygen, nitrogen, sulfur, silicon, phosphorus, boron, and the like either may be present in the alkylene group). The alkylene group for R₁ includes from 1 carbon atom to 12 carbon atoms. In another embodiment, the alkylene group for R₁ includes no more than 4 carbon atoms, and in yet another embodiment no more than 2 carbon atoms.

The arylene group for R₁ is defined as a divalent aromatic group or aryl group, including substituted and unsubstituted arylene groups, and wherein heteroatoms, such as oxygen, nitrogen, sulfur, silicon, phosphorus, boron, and the like either may be present in the arylene group. The arylene group for R₁ includes from 5 carbon atoms to 14 carbon atoms. In another embodiment, the arylene group for R₁ includes no more than 10 carbon atoms, and in yet another embodiment with no more than 6 carbon atoms.

The arylalkylene group for R₁ is defined as a divalent arylalkyl group, including substituted and unsubstituted arylalkylene groups, wherein the alkyl portion of the arylalkylene group can be linear or branched, saturated or unsaturated, and cyclic or acyclic, and wherein heteroatoms, such as oxygen, nitrogen, sulfur, silicon, phosphorus, boron, and the like either may be present in either the aryl or the alkyl portion of the arylalkylene group. The arylalkylene group for R₁ includes at least from 6 carbon atoms, and in another embodiment with at least 7 carbon atoms. In one embodiment, the arylalkylene group for R₁ includes no more than 32 carbon atoms, in another embodiment with no more than 22 carbon atoms, and in yet another embodiment with no more than 7 carbon atoms.

The alkylarylene group for R₁ is defined as a divalent alkylaryl group. including substituted and unsubstituted alkylarylene groups, wherein the alkyl portion of the alkylarylene group can be linear or branched, saturated or unsaturated, and cyclic or acyclic, and wherein heteroatoms, such as oxygen, nitrogen, sulfur, silicon, phosphorus, boron, and the like either may or may not be present in either the aryl or the alkyl portion of the alkylarylene group. The alkylarylene group for R₁ includes at least 6 carbon atoms, and in another embodiment with at least 7 carbon atoms. In one embodiment, the alkylarylene group for R₁ includes no more than 32 carbon atoms, in another embodiment with no more than 22 carbon atoms, and in yet another embodiment with no more than 7 carbon atom. Furthermore, the substituents on the substituted alkylene, arylene, arylalkylene, and alkylarylene groups can be halogen atoms, cyano groups, pyridine groups, pyridinium groups, ether groups, aldehyde groups, ketone groups, ester groups, amide groups, carbonyl groups, thiocarbonyl groups, sulfide groups, nitro groups, nitroso groups, acyl groups, azo groups, urethane groups, urea groups, mixtures thereof, and the like, wherein two or more substituents can be joined together to form a ring.

The alkylene group for R₂ and R₂' may include a divalent aliphatic group or alkyl group, including linear and branched, saturated and unsaturated, cyclic and acyclic, and substituted and unsubstituted alkylene groups, and wherein heteroatoms, such as oxygen, nitrogen, sulfur, silicon, phosphorus, boron, and the like either may or may not be present in the alkylene group). The alkylene group for R₂ and R₂' includes at least I carbon atom, and in one embodiment with no more than 54 carbon atoms, and in another embodiment with no more than 36 carbon atoms.

The arylene group for R₂ and R₂' may include a divalent aromatic group or aryl group, including substituted and unsubstituted arylene groups, and wherein heteroatoms, such as oxygen, nitrogen, sulfur, silicon, phosphorus, boron, and the like either may or may not be present in the arylene group. The arylene group for R₂ and R₂' includes at least 5 carbon atoms, and in one embodiment with no more than 14 carbon atoms, in another embodiment with no more than 10 carbon atoms, and in yet another embodiment with no more than 7 carbon atoms.

The arylalkylene group for R₂ and R₂' may include a divalent arylalkyl group, including substituted and unsubstituted arylalkylene groups, wherein the alkyl portion of the arylalkylene group can be linear or branched, saturated or unsaturated, and cyclic or acyclic, and wherein heteroatoms, such as oxygen, nitrogen, sulfur, silicon, phosphorus, boron, and the like either may or may not be present in either the aryl or the alkyl portion of the arylalkylene group. The arylalkylene group for R₂ and R₂' includes at least 6 carbon atoms, and in one embodiment with no more than 32 carbon atoms, in another embodiment with no more than 22 carbon atoms, and in yet another embodiment with no more than 8 carbon atoms.

The alkylarylene group for R₂ and R₂' may include a divalent alkylaryl group, including substituted and unsubstituted alkylarylene groups, wherein the alkyl portion of the alkylarylene group can be linear or branched, saturated or unsaturated, and cyclic or acyclic, and wherein heteroatoms, such as oxygen, nitrogen, sulfur, silicon, phosphorus, boron, and the like either may or may not be present in either the aryl or the alkyl portion of the alkylarylene group. The alkylarylene group for R₂ and R₂' includes at least 6 carbon atoms, and in one embodiment with no more than 32 carbon atoms, in another embodiment with no more than 22 carbon atoms, and in yet another embodiment with no more than 7 carbon atoms, although the number of carbon atoms can be outside of these ranges. The substituents for the alkylene, arylene, arylalkylene, and alkylarylene groups can be (but are not limited to) halogen atoms, cyano groups, ether groups, aldehyde groups, ketone groups, ester groups; amide groups, carbonyl groups, thiocarbonyl groups, phosphine groups, phosphonium groups, phosphate groups, nitrile groups, mercapto groups, nitro groups, nitroso groups, acyl groups, acid anhydride groups, azide groups, azo groups, cyanato groups, urethane groups, urea groups, mixtures thereof, and the like, wherein two or more substituents can be joined together to form a ring.

The alkylarylene group for R₂ may be derived from 1-(4-(2-hydroxyethoxy)phenyl)-2-hydroxy-2-methylpropan-1-one, 1-hydroxycyclohexylphenylketone, 2-hydroxy-2-methyl-1-phenylpropan-1-one, and the like. The formulas for these compounds are described in paragraph [0073] of U.S. Patent Application Pub. No. 2008/0218570.

The alkyl group for R₃ and R₃' may include linear and branched, saturated and unsaturated, cyclic and acyclic, and substituted and unsubstituted alkyl groups, and wherein heteroatoms, such as oxygen, nitrogen, sulfur, silicon, phosphorus, boron, and the like either may be present in the alkyl group. The alkyl group for R₃ and R₃' includes at least 2 carbon atoms, in another embodiment with at least 3 carbon atoms, and in yet another embodiment with at least 4 carbon atoms, and in one embodiment with no more than 100 carbon atoms, in another embodiment with no more than 60 carbon atoms, and in yet another embodiment with no more than 30 carbon atoms.

The alkyl group for R₃ and R₃' may include substituted and unsubstituted aryl groups, and wherein heteroatoms, such as oxygen, nitrogen, sulfur, silicon, phosphorus, boron, and the like either may be present in the aryl group. The aryl group for R₃ includes at least 5 carbon atoms, and in another embodiment with at least 6 carbon atoms, and in one embodiment with no more than 100 carbon atoms, in another embodiment with no more than 60 carbon atoms, and in yet another embodiment with no more than 30 carbon atoms.

The arylalkyl group for R₃ and R₃' may include a substituted and unsubstituted arylalkyl groups, wherein the alkyl portion of the arylalkyl group can be linear or branched, saturated or unsaturated, and cyclic or acyclic, and wherein heteroatoms, such as oxygen, nitrogen, sulfur, silicon, phosphorus, boron, and the like either may be present in either the aryl or the alkyl portion of the arylalkyl group. The arylalkyl group for R₃ and R₃' includes at least 6 carbon atoms, and in another embodiment at least 7 carbon atoms, and in one embodiment no more than 100 carbon atoms, in another embodiment no more than 60 carbon atoms, and in yet another embodiment no more than 30 carbon atoms.

The alkylaryl group for R₃ and R₃' may include substituted and unsubstituted alkylaryl groups, wherein the alkyl portion of the alkylaryl group can be linear or branched, saturated or unsaturated, and cyclic or acyclic, and wherein heteroatoms, such as oxygen, nitrogen, sulfur, silicon, phosphorus, boron, and the like either may be present in either the aryl or the alkyl portion of the alkylaryl group. The alkylaryl group for R₃ and R₃' includes at least 6 carbon atoms, and in another embodiment at least 7 carbon atoms, and in one embodiment no more than 100 carbon atoms, in another embodiment with no more than 60 carbon atoms, and in yet another embodiment with no more than 30 carbon atoms, although the number of carbon atoms can be outside of these ranges, such as tolyl or the like. The substituents on the substituted alkyl, arylalkyl, and alkylaryl groups can be halogen atoms, ether groups, aldehyde groups, ketone groups, ester groups, amide groups, carbonyl groups, thiocarbonyl groups, sulfate groups, sulfonate groups, sulfonic acid groups, sulfide groups, sulfoxide groups, phosphine groups, phosphonium groups, phosphate groups, nitrile groups, mercapto groups, nitro groups, nitroso groups, sulfone groups, acyl groups, acid anhydride groups, azide groups, azo groups, cyanato groups, isocyanato groups, thiocyanato groups, isothiocyanato groups, carboxylate groups, carboxylic acid groups, urethane groups, urea groups, mixtures thereof, and the like, wherein two or more substituents can be joined together to form a ring.

The X and X' may include an oxygen atom or a group of the formula --NR₄--, wherein R₄ is: (i) a hydrogen atom; (ii) an alkyl group, including linear and branched, saturated and unsaturated, cyclic and acyclic, and substituted and unsubstituted alkyl groups, and wherein heteroatoms either may be present in the alkyl group, in one embodiment with at least I carbon atom, and in one embodiment with no more than 100 carbon atoms, in another embodiment with no more than 60 carbon atoms, and in yet another embodiment with no more than 30 carbon atoms, (iii) an aryl group, including substituted and unsubstituted aryl groups, and wherein heteroatoms either may be present in the aryl group, in one embodiment with at least 5 carbon atoms, and in another embodiment with at least 6 carbon atoms, and in one embodiment with no more than 100 carbon atoms, in another embodiment with no more than 60 carbon atoms, and in yet another embodiment with no more than 30 carbon atoms, (iv) an arylalkyl group, including substituted and unsubstituted arylalkyl groups, wherein the alkyl portion of the arylalkyl group can be linear or branched, saturated or unsaturated, and cyclic or acyclic, and wherein heteroatoms either may be present in either the aryl or the alkyl portion of the arylalkyl group, in one embodiment with at least 6 carbon atoms, and in another embodiment with at least 7 carbon atoms, and in one embodiment with no more than 100 carbon atoms, in another embodiment with no more than 60 carbon atoms, and in yet another embodiment with no more than 30 carbon atoms, or (v) an alkylaryl group, including substituted and unsubstituted alkylaryl groups, wherein the alkyl portion of the alkylaryl group can be linear or branched, saturated or unsaturated, and cyclic or acyclic, and wherein heteroatoms either may be present in either the aryl or the alkyl portion of the alkylaryl group, in one embodiment with at least 6 carbon atoms, and in another embodiment with at least 7 carbon atoms, and in one embodiment with no more than 100 carbon atoms, in another embodiment with no more than 60 carbon atoms, and in yet another embodiment with no more than 30 carbon atoms, , wherein the substituents on the substituted alkyl, aryl, arylalkyl, and alkylaryl groups can be (but are not limited to) halogen atoms, ether groups, aldehyde groups, ketone groups, ester groups, amide groups, carbonyl groups, thiocarbonyl groups, sulfate groups, sulfonate groups, sulfonic acid groups, sulfide groups, sulfoxide groups, phosphine groups, phosphonium groups, phosphate groups, nitrile groups, mercapto groups, nitro groups, nitroso groups, sulfone groups, acyl groups, acid anhydride groups, azide groups, azo groups, cyanato groups, isocyanato groups, thiocyanato groups, isothiocyanato groups, carboxylate groups, carboxylic acid groups, urethane groups, urea groups, mixtures thereof, and the like, wherein two or more substituents can be joined together to form a ring.

In specific embodiments, the gellant is a compound of one of the formulas described in U.S. Patent Application Pub. No. 2008/0218570. The gellant compounds as disclosed herein can be prepared by any desired or effective method, including by not limited to the method described U.S. Patent Application Pub. No. 2008/0218570.

Furthermore, some of the curable monomers described above may also a exhibit gel-like behavior in that they undergo a relatively sharp increase in viscosity over a relatively narrow temperature range when dissolved in a liquid. One example of such a liquid monomer is a propoxylated neopentyl glycol diacrylate such as SR9003. commercially available from Sartomer Co. Inc.

The ink compositions can include a gellant in any suitable amount, such as from 1% to 50% by weight of the ink. In embodiments, the gellant can be present in an amount of 2% to 20% by weight of the ink and such as 5% to 15% by weight of the ink.

A curable wax may also be used as a phase change agent. The curable wax may be any wax component that is miscible with the other components and that will polymerize with the curable monomer to form a polymer. The term "wax" includes, for example, any of the various natural, modified natural, and synthetic materials commonly referred to as waxes. A wax is solid at room temperature, specifically at 25°C and may promote an increase in viscosity of the ink as it cools from the jetting temperature.

Suitable examples of curable waxes include those waxes that include or are functionalized with curable groups. The curable groups may include, for example, acrylate, methacrylate, alkene, allylic ether, epoxide, oxetane, and the like. These waxes can be synthesized by the reaction of a wax equipped with a transformable functional group, such as carboxylic acid or hydroxyl.

Suitable examples of hydroxyl-terminated polyethylene waxes that may be functionalized with a curable group include, but are not limited to, mixtures of carbon chains with the structure CH₃-(CH₂)ₙ-CH₂OH, where n is the chain length and can be in the range of 16 to 50, from 20 to 40, from 25 to 35 and from 25 to 30.

Suitable examples of carboxylic acid-terminated polyethylene waxes that may be functionalized with a curable group include mixtures of carbon chains with the structure CH₃-(CH₂)ₙ-COOH, where n is the chain length and can be in the range of 16 to 50, from 20 to 40, from 25 to 35 and from 25 to about 30.

Other suitable examples of curable waxes include, for example, AB₂ diacrylate hydrocarbon compounds that may be prepared by reacting AB₂ molecules with acryloyl halides, and then further reacting with aliphatic long-chain, mono-functional aliphatic compounds. Suitable functional groups useful as A groups in embodiments include carboxylic acid groups and the like. Suitable functional groups useful as B groups in embodiments may be hydroxyl groups, thiol groups, amine groups, amide groups, imide groups, phenol groups, and mixtures thereof.

The curable wax can be included in the ink composition in an amount of from 0 to 25% by weight of the ink, such as, for example, from 1 to 15% by weight of ink and from 2 to 10 by weight of the ink. In an embodiment, the curable wax can be included in the ink composition in an amount of from 3 to 10% by weight of the ink, such as 4 to 6% by weight of the ink.

The radiation curable phase change inks may also contain an optional colorant. Any desired or effective colorant can be employed in the inks, including pigment, dye, mixtures of pigment and dye, mixtures of pigments, mixtures of dyes, and the like, provided that the colorant can be dissolved or dispersed in the ink vehicle.

The colorant may be present in the phase change ink in any desired or effective amount to obtain the desired color or hue such as, for example, from 0 percent by weight of the ink to 50 percent by weight of the ink, at least from 0.2 percent by weight of the ink to 20 percent by weight of the ink, and at least from 0.5 percent by weight of the ink to 10 percent by weight of the ink.

In embodiments, the radiation curable phase change inks may further comprise an initiator, such as a photoinitiator, that initiates polymerization of curable components of the ink, including the curable monomer and the optional curable wax. The initiator should be soluble in the composition. In embodiments, the initiator is an ultraviolet-activated (UV-activated) photoinitiator.

In embodiments, the initiator can be a radical initiator. Examples of radical photoinitiators include benzophenone derivatives, benzyl ketones, monomeric hydroxyl ketones, alpha.-amino ketones, acyl phosphine oxides, metallocenes, benzoin ethers, benzil ketals, alpha.-hydroxyalkylphenones, alpha.-aminoalkylphenones, acylphosphine photoinitiators sold under the trade designations of IRGACURE and DAROCUR from Ciba, isopropyl thioxanthenones, and the like, and combinations thereof.

The radiation curable phase change inks may also contain an amine synergist. An amine synergist is a co-initiator that donates a hydrogen atom to a photoinitiator and thereby forms a radical species that initiates polymerization (amine synergists can also consume oxygen dissolved in the ink--as oxygen inhibits free radical polymerization its consumption increases the speed of polymerization). Examples of the amine synergists may include ethyl-4-dimethylaminobenzoate and 2-ethylhexyl-4-dimethylaminobenzoate.

In other embodiments, the initiator can be a cationic initiator. Examples of suitable cationic photoinitiators may include aryldiazonium salts, diaryliodonium salts, triarysulfonium salts, triarylselenonium salts, dialkylphenacylsulfonium salts, triarylsulphoxonium salts and aryloxydiarylsulfonium salts.

Initiators that absorb radiation, for example UV light radiation, to initiate curing of the curable components of the ink may also be used. Examples of initiators absorb radiation at any desired or effective wavelength, for example, from 200 to 600 nanometers, from 200 to 500 nanometers, and from 200 to 420 nanometers. The total amount of initiator included in the ink may be, for example, from 0.5% to 15%, and from 1% to 10%, by weight of the ink.

The radiation curable phase change inks can also optionally contain an antioxidant. The optional antioxidants can protect the images from oxidation and can also protect the ink components from oxidation during the heating portion of the ink preparation process.

When present, the optional antioxidant is present in the ink in any desired or effective amount, for example from at least 0.01 percent by weight of the ink carrier to 20 percent by weight of the ink carrier, from 0.1 percent by weight of the ink carrier to 5 percent by weight of the ink carrier, and from 1 percent by weight of the ink carrier to 3 percent by weight of the ink carrier.

The radiation curable phase change inks can also contain additives to take advantage of the known functionality associated with such additives. Such additives may include, for example, defoamers, slip and leveling agents, pigment dispersants, and the like, as well as mixtures thereof.

In one specific embodiment, the inks are jetted at low temperatures, such as temperatures below 10°C, from 40°C to 110°C, from 50°C to 110°C, and from 60°C to 90°C. At such low jetting temperatures, the temperature differential between the jetted ink and the flexographic plate upon which the ink is jetted can be used to rapidly effect a phase change in the ink (that is, from liquid to solid) due to the inclusion of the phase change agent.

In some embodiments, the gel point temperature at which the ink forms the gel state is any temperature below the jetting temperature of the ink, in one embodiment any temperature that is 5°C or more below the jetting temperature of the ink. In one embodiment, the gel state can be formed as the temperature drops to a temperature of at least 25°C, and in another embodiment at a temperature of at least 30°C, and in one embodiment of no more than 100°C, in another embodiment of no more than 70°C, and in yet another embodiment of no more than 50°C, although the temperature can be outside of these ranges. A rapid and large increase in ink viscosity occurs upon cooling from the jetting temperature, at which the ink is in a liquid state, to the gel point temperature, at which the ink is in the gel state.

The phase change ink compositions can be prepared by any desired or suitable method. For example, the ink ingredients can be mixed together, followed by heating, to a temperature in one embodiment of from 80°C to 120°C, and stirring until a homogeneous ink composition is obtained, followed by cooling the ink to ambient temperature, for example from 20°C to 25°C. The inks are solid at ambient temperature.

The inks can be employed in an apparatus or a device for direct printing ink jet processes and in indirect (offset) printing ink jet applications. A direct printing process is also disclosed in, for example, U.S. Pat. No. 5,195,430. In embodiments, disclosed herein is directed to a process which comprises incorporating an ink as disclosed herein into an ink jet printing apparatus, melting the ink, forming a first ink layer by causing droplets of the melted ink to be ejected in an imagewise pattern onto a flexographic plate and gelling ink; forming additional ink layer on top of the first ink layer until a flexographic print master with a sufficient thickness is formed.

Upon deposition onto the flexographic plate, the radiation curable phase change ink, which was ejected from the inkjet printhead as a liquid, solidifies into a gel on the flexographic plate. The phase transition allows for high image quality which can be achieved without the need for pinning.

Thus, printing on a flexographic plate may comprise providing and heating a radiation-curable phase change ink. Heating the phase change ink generally causes the ink to become liquid. The ink is then jetted from a printhead onto a flexographic plate one time to form the first layer of the pattern of the image. Upon deposition, each layer of the ink is cooled and gels on the surface of the flexographic plate (due to the difference in temperature), which causes a phase change back to a semi-solid gel. Each subsequent layer is jetted only after the previously jetted layer gels. This gelling may occur very rapidly, for example, in less than one second, so that the additional layers can be deposited directly on top of the first layer to form a printing master with a raised surface. The additional layers may be formed using a printhead to jet the ink for 1 to 100 times, from 5 to 40 times, from 10 to 40 times and from 20 to 30 times, until a printing master with sufficient thickness is formed. The thickness of each layer in the printing master may have a thickness of at least one drop of the melted ink.

The thickness of the printing master may be from 0.01 mm to 100 mm, from 0.05 mm to 1 mm, from 0.1 mm to 1 mm and from 0.5 mm to 1 mm. Finally, the ink is cured in the ambient atmosphere each layer of the printing master is formed.

The printing master with a raised surface can be formed into a three dimensional image, such as for example, a letter, a number or a symbol. The pattern for the printing master may have a straight edge or a tapered edge.

In embodiments, after a sufficient number of ink layers have been deposited on the flexographic plate, will the ink layers are cured. Thus, the single-step cure allows the printing master to be produced much quicker.

In embodiments, the printing master may also be produced by more than one curing step. For example, an initial portion of the printing master comprised of gelled layers may be formed on the flexographic plate. The initial portion represents at least 5% percent of the desired thickness for the printing master, such as, for example, from 5% to 60%, from 10% to 50% from 15% to 40% and from 20% to 35%, of the desired thickness of the printing master. After the initial portion of the printing master is cured, additional post-initial curing layers are deposited on top of the initial curing portion and gelled. Upon curing, these post-initial curing layers comprise the remaining thickness necessary to achieve the desired or sufficient thickness of the printing master. The printing master may also be produced by multiple additional deposition and curing steps.

Curing is defined when the curable compounds in the ink undergo an increase in molecular weight upon exposure to actinic radiation, such as crosslinking, chain lengthening, or the like that results in a hardening of the ink. Curing of the ink can be effected by exposure of the ink image to ultraviolet radiation or actinic radiation for any desired or effective period of time, such as, for example, from 0.01 seconds to 30 seconds, from 0.01 seconds to 15 seconds, and from 0.01 seconds to 5 seconds.

Actinic radiation sources encompass the ultraviolet and visible wavelength regions. The suitability of a particular actinic radiation source is governed by the photosensitivity of the initiator and the monomers used in preparing the flexographic printing masters. The preferred photosensitivity of most common flexographic printing masters are in the UV and deep UV area of the spectrum, as they afford better room-light stability. Examples of suitable visible and UV sources include carbon arcs, mercury-vapor arcs, fluorescent lamps, electron flash units, electron beam units, lasers, and photographic flood lamps.

Any ultraviolet light source may be employed as a radiation source, such as, for example, a high or low pressure mercury lamp, a cold cathode tube, a black light, an ultraviolet LED, an ultraviolet laser, and a flash light. Furthermore, the ultraviolet light source may be a radiation source that exhibits a relatively long wavelength UV-contribution having a dominant wavelength of 300-400 nm. Specifically, a UV-A (320 nm to 400 nm) light source may also be used due to the reduced light scattering therewith resulting in more efficient interior curing. However, UV-B (290 nm to 320 nm) or UV-C (100 nm to 290 nm) may also be used.

Examples of suitable materials for the support for the flexographic plate include transparent polymeric films such those formed by addition polymers and linear condensation polymers, transparent foams and fabrics. Under certain end-use conditions, metals such as steel, aluminum, copper and nickel, although not transparent, may also be used as a plate. The support may be in sheet form or in cylindrical form, such as a sleeve. The sleeve may be formed from single layer or multiple layers of flexible material, as for example disclosed by U.S. Patent Application Pub. No. 2002/0046668_{.} Flexible sleeves made of polymeric films or multiple layered sleeves, such as those described in U.S. Patent No. 5.301,610 may also be used. The sleeve may also be made of non-transparent, actinic radiation blocking materials, such as nickel or glass epoxy.

The support may have a thickness from 0.002 to 0.050 inch (0.0051 to 0.127 cm). A preferred thickness for the sheet form is 0.003 to 0.016 inch (0.0076 to 0.040 cm). The sleeve typically has a wall thickness from 10 to 80 mils (0.025 to 0.203 cm) or more. Preferred wall thickness for the cylinder form is 10 to 40 mils (0.025 to 0.10 cm).

### EXAMPLES

### Example 1 (colorless ink)

A solution is formed in a 600 mL beaker by adding (a) 400 g of SR9003^{®} (dimer acrylate), (b) 27.5 g of SR399LV (pentafunctional acrylate) and (c) a mixture of phtoinitiators comprised of 19.5 g of IRGACURE 127^{®}, 16.5 g of IRGACURE 379^{®}, 5.5 g of IRGACURE 819^{®} and 11 g of DAROCURE ITX^{®}. The resulting solution is heated to 90°C, at which time 27.5 grams of UNILIN 350^{®} (acrylate wax) and 41.25 g of a UV curable gellant are added to form a mixture. Upon stirring the mixture for 3 hours, the mixture is filtered to produce a colorless ink composition.

### Example 2 (colored ink)

A solution is formed in a 600 mL beaker by adding (a) 400 g of SR9003^{®} (dimer acrylate), (b) 27.5 g of SR399LV^{®} (pentafunctional acrylate) and (c) a mixture of photoinitiators comprised of 19.5 g of IRGACURE 127^{®}, 16.5 g of IRGACURE 379^{®}, 5.5 g of IRGACURE 819^{®} and 11 g of DAROCURE ITX^{®}. The resulting solution is heated to 90°C, at which time 27.5 grams of UNILIN 350^{®} acrylate wax and 41.25 g of a UV curable gellant are added to form a mixture. Upon stirring for 3 hours and subsequently filtering the mixture, 110 g of a 3% dispersion of cyan pigment is added at 90°C and continuously heated at this temperature for 3 hours. The colored solution is then filtered to produce a cyan ink composition.

### Printing of Example 1

The ink is heated to a temperature greater than 80°C to produce a melted ink. The melted ink is then placed in a printhead that is at a temperature greater than 80°C. The melted ink is then jetted onto a rigid polymer, wherein the gellant in the ink composition forms layers of a relief image. The relief image is then cured upon exposure to ultraviolet light. The cured relief image results in a three-dimensional structure with a thickness of from 300pm that can be used as a flexographic printing master.

## Claims

1. A method of forming a printing master on a flexographic plate, the method comprising:
(a) melting a radiation-curable phase change ink comprised of at least one curable monomer, at least one phase change agent, at least one photoinitiator and an optional colorant,
(b) depositing multiple layers of the melted ink at desired locations on the flexographic plate to form a raised pattern, wherein each deposited layer of ink is gelled prior to the deposition of a subsequent layer on the deposited layer, until the printing master with sufficient thickness is formed on the flexographic plate, and
(c) curing the ink on the flexographic plate upon the conclusion of the depositing step.

2. The method of claim 1, wherein the phase change agent is a gellant.

3. The method of claim 1 or 2, wherein the ink is cured by exposing the ink to ultraviolet radiation.

4. The method of any of claims 1 to 3, wherein the viscosity of the melted ink is from 0.001 to 100 Pa·s (10⁰ cP to 10⁵ cP) at a temperature of from 60°C to 100°C.

5. The method of any of claims 1 to 4, wherein the deposition of the ink for the deposited multiple layers occurs in a single pass of a printing device.

6. The method of any of claims 1 to 5, wherein the thickness of the deposited multiple layers is from 0.01 mm to 100 mm.

7. The method of any of claims 1 to 6, wherein the melted ink is deposited by jetting the melted ink from a printing device for 1 to 100 times to form the deposited multiple layers.

8. A method of forming a printing master on a flexographic plate, the method comprising:
(a) melting a radiation-curable phase change ink comprised of at least one curable monomer, at least one gellant, at least one photoinitiator and an optional colorant,
(b) depositing the melted ink on the flexographic plate in a pattern to form a layer of the pattern,
(c) allowing the deposited layer of the ink to gel on the flexographic plate,
(d) depositing the melted ink on the previous deposited layer to form an additional layer,
(e) allowing the deposited additional layer to gel,
(f) repeating steps (d) through (e) to form further additional deposited and gelled layers, until the printing master with sufficient thickness is formed on the flexographic plate, and
(g) curing the ink on the flexographic plate upon the achievement of the sufficient thickness,
(h) wherein the viscosity of the melted ink is from 0.001 to 100 Pa·s (10⁰ cP to 10⁵ cP) at a temperature of from 60°C to 100°C.

9. The method of claim 8, wherein the ink is cured by exposing the ink to ultraviolet radiation.

10. The method of claim 8 or 9, wherein the deposition of the ink for the deposited layer occurs in a single pass of a printing device.

11. The method of any of claims 8 to 10, wherein the deposition of the ink for the additional deposited layer and the further additional deposited layer occurs in a single pass of a printing device.

12. The method of any of claims 8 to 11, wherein a total thickness of the deposited layer, the deposited additional layer and the further additional deposited layers is from 0.01 mm to 100 mm.

13. The method of any of claims 8 to 12, wherein the melted ink is deposited by jetting the melted ink from a printing device a single time to form deposited layer and the deposited additional layer.

14. A method of forming a printing master on a flexographic plate, the method comprising:
(a) melting a radiation-curable phase change ink comprised of at least one curable monomer, at least one phase change agent, at least one photoinitiator and an optional colorant,
(b) depositing the melted ink on the flexographic plate in a pattern to form a layer in the pattern,
(c) allowing the deposited layer of the ink to gel on the flexographic plate,
(d) depositing an additional layer of the melted ink on the previous deposited layer,
(e) allowing the deposited additional layer to gel,
(f) repeating steps (d) through (e) to form further additional deposited and gelled layers, until the printing master with an initial thickness is formed on the flexographic plate,
(g) curing the ink on the flexographic plate to form an initial portion of the printing master,
(h) depositing a post-initial curing layer of the melted ink on the initial portion of the printing master,
(i) allowing the deposited post-initial curing layer of the melted ink to gel on the flexographic plate,
(j) depositing an additional post-initial curing layer of the melted ink on the previous deposited post-initial curing layer,
(k) allowing the deposited additional post-initial curing layer to gel,
(l) repeating steps (j) through (k) to form further additional post-initial curing deposited and gelled layers, until the printing master with sufficient thickness is formed on the flexographic plate, and
(m) curing the ink on the flexographic plate upon the achievement of the sufficient thickness.

15. The method of claim 14, wherein the initial thickness of the printing master is from 5 to 60 percent of the sufficient thickness.

## Patentansprüche

1. Verfahren zum Formen einer Druckschablone auf einer flexographischen Platte, wobei das Verfahren umfasst:
(a) Schmelzen einer durch Strahlung härtbaren Phasenaustauschtinte umfassend wenigstens ein härtbares Monomer, wenigstens ein Phasenaustauschmittel, wenigstens einen Photoinitiator und gegebenenfalls einen Farbstoff,
(b) Abscheiden einer Vielzahl von Schichten aus geschmolzener Tinte auf gewünschte Bereichen der flexographischen Platte, um ein erhobenes Muster zu bilden, wobei jede abgeschiedene Tintenschicht vor der Abscheidung einer nachfolgenden Schicht auf der abgeschiedenen Schicht geliert wird, bis die Druckschablone mit ausreichender Dicke auf der flexographischen Platte geformt ist, und
(c) Härten der Tinte auf der flexographischen Platte nach Abschluss des Abscheidungsschrittes.

2. Verfahren nach Anspruch 1, wobei das Phasenaustauschmittel ein Geliermittel ist.

3. Verfahren nach Anspruch 1 oder 2, wobei die Tinte gehärtet wird, indem die Tinte ultravioletter Strahlung ausgesetzt wird.

4. Verfahren nach einem der Ansprüche 1 bis 3, wobei die Viskosität der geschmolzenen Tinte zwischen 0,001 bis 100 Pa·s (10⁰ cP bis 10⁵ cP) bei einer Temperatur von 60°C bis 100°C beträgt.

5. Verfahren nach einem der Ansprüche 1 bis 4, wobei die Abscheidung der Tinte für die abgeschiedenen mehrfachen Schichten in einem einzelnen Durchgang einer Druckvorrichtung erfolgt.

6. Verfahren nach einem der Ansprüche 1 bis 5, wobei die Dicke der abgeschiedenen Mehrschichtfilme von 0,01 mm bis 100 mm beträgt.

7. Verfahren nach einem der Ansprüche 1 bis 6, wobei die geschmolzene Tinte durch Ausstoßen der geschmolzenen Tinte aus einer Druckvorrichtung 1 bis 100 Mal abgeschieden wird, um die abgeschiedenen Mehrfachschichten zu bilden.

8. Verfahren zum Formen einer Druckschablone auf einer flexograpischen Platte, wobei das Verfahren umfasst:
(a) Schmelzen einer durch Bestrahlung härtbaren Phasenaustauschtinte umfassend wenigstens ein härtbares Monomer, wenigstens ein Geliermittel, wenigstens einen Photoinitiator und gegebenenfalls einen Farbstoff,
(b) Abscheiden der geschmolzenen Tinte auf der flexographischen Platte in einem Muster, um eine Musterschicht zu formen,
(c) Ermöglichen, dass die abgeschiedene Tintenschicht auf der flexographischen Platte geliert,
(d) Abscheiden der geschmolzenen Tinte auf der zuvor abgeschiedenen Schicht, um eine zusätzliche Schicht zu bilden,
(e) Ermöglichen, dass die zusätzliche abgeschiedene Schicht geliert,
(f) Wiederholen der Schritte (d) bis (e), um weitere zusätzliche abgeschiedene und gelierte Schichten zu bilden, bis die Druckschablone mit ausreichender Dicke auf der flexographischen Platte geformt ist, und
(g) Härten der Tinte auf der flexographischen Platte bei Erzielung der ausreichenden Dicke,
(h) wobei die Viskosität der geschmolzenen Tinte von 0,001 bis 100 Pa·s (10⁰ cP bis 10⁵ cP) bei einer Temperatur von 60°C bis 100°C beträgt.

9. Verfahren nach Anspruch 8, wobei die Tinte gehärtet wird, indem die Tinte ultravioletter Strahlung ausgesetzt wird.

10. Verfahren nach Anspruch 8 oder 9, wobei das Abscheiden der Tinte für die abgeschiedenen Schichten in einem einzelnen Durchgang einer Druckvorrichtung stattfindet.

11. Verfahren nach einem der Ansprüche 8 bis 10, wobei die Abscheidung der Tinte für die zusätzlich abgeschiedene Schicht und die weitere zusätzlich abgeschiedene Schicht in einem einzelnen Durchgang einer Druckvorrichtung erfolgt.

12. Verfahren nach einem der Ansprüche 8 bis 11, wobei eine Gesamtdicke der abgeschiedenen Schicht, der abgeschiedenen zusätzlichen Schicht und der weiteren zusätzlichen abgeschiedenen Schichten von 0,01 mm bis 100 mm beträgt.

13. Verfahren nach einem der Ansprüche 8 bis 12, wobei die geschmolzene Tinte durch Ausstoßen der geschmolzenen Tinte aus einer Druckeinrichtung ein einziges Mal abgeschieden wird, um die abgeschiedene Schicht und die abgeschiedene zusätzliche Schicht zu bilden.

14. Verfahren zur Herstellung einer Druckschablone auf einer flexographischen Platte, wobei das Verfahren umfasst:
(a) Schmelzen einer durch Bestrahlung härtbaren Phasenaustauschtinte umfassend wenigstens ein härtbares Monomer, wenigstens ein Phasenaustauschmittel, wenigstens ein Photoinitiator und gegebenenfalls einen Farbstoff,
(b) Abscheiden der geschmolzenen Tinte auf der flexographischen Platte in einem Muster, um eine Schicht in dem Muster zu bilden,
(c) Ermöglichen, dass die abgeschiedene Schicht der Tinte auf der flexographischen Platte geliert,
(d) Abscheiden einer zusätzlichen Schicht der geschmolzenen Tinte auf der zuvor abgeschiedenen Schicht,
(e) Ermöglichen, dass die abgeschiedene zusätzliche Schicht geliert,
(f) Wiederholen der Schritte (d) bis (e), um weitere zusätzliche abgeschiedene und gelierte Schichten zu bilden, bis die Druckschablone mit einer initialen Dicke auf der flexographischen Platte gebildet ist,
(g) Härten der Tinte auf der flexographischen Platte, um einen initialen Bereich der Druckschablone zu bilden,
(h) Abscheiden einer postinitialen Härtungschicht der geschmolzenen Tinte auf dem initialen Bereich der Druckschablone,
(i) Ermöglichen, dass die abgeschiedene postinitiale Härtungsschicht der geschmolzenen Tinte auf der flexographischen Platte geliert,
(j) Abscheiden einer zusätzlichen postinitialen Härtungsschicht auf der geschmolzenen Tinte auf der zuvor abgeschiedenen postinitialen Härtungsschicht,
(k) Ermöglichen, dass die abgeschiedene zusätzliche postinitiale Härtungsschicht geliert,
(l) Wiederholen der Schritte (j) bis (k), um weitere zusätzliche postinitiale abgeschiedene gelierte Härtungsschichten zu bilden, bis die Druckschablone mit ausreichender Dicke auf der flexographischen Platte geformt ist, und
(m) Härten der Tinte auf der flexographischen Platte nach Erzielung der ausreichenden Dicke.

15. Verfahren nach Anspruch 14, wobei die initale Dicke der Druckschablone zwischen 5 bis 60% der ausreichenden Dicke beträgt.

## Revendications

1. Procédé de formation d'un original d'impression sur une plaque flexographique, le procédé comprenant le fait :
(a) de faire fondre une encre à changement de phase durcissable par rayonnement composée d'au moins un monomère durcissable, d'au moins un agent de changement de phase, d'au moins un photo-initiateur et d'un colorant facultatif,
(b) de déposer plusieurs couches de l'encre fondue à des emplacements souhaités sur la plaque flexographique pour former un motif en relief, où chaque couche d'encre déposée est gélifiée avant le dépôt d'une couche suivante sur la couche déposée, jusqu'à ce que l'original d'impression avec une épaisseur suffisante soit formé sur la plaque flexographique, et
(c) de durcir l'encre sur la plaque flexographique à la fin de l'étape de dépôt.

2. Procédé de la revendication 1, dans lequel l'agent de changement de phase est un gélifiant.

3. Procédé de la revendication 1 ou 2, dans lequel l'encre est durcie par l'exposition de l'encre aux rayons ultraviolets.

4. Procédé de l'une des revendications 1 à 3, dans lequel la viscosité de l'encre fondue est de 0,001 à 100 Pa·s (10⁰ cP à 10⁵ cP) à une température allant de 60°C à 100°C.

5. Procédé de l'une des revendications 1 à 4, dans lequel le dépôt de l'encre pour la pluralité de couches déposées se produit en un seul passage d'un dispositif d'impression.

6. Procédé de l'une des revendications 1 à 5, dans lequel l'épaisseur de la pluralité de couches déposées va de 0,01 mm à 100 mm.

7. Procédé de l'une des revendications 1 à 6, dans lequel l'encre fondue est déposée par jet entre 1 à 100 fois de l'encre fondue à partir d'un dispositif d'impression afin de former plusieurs couches déposées.

8. Procédé de formation d'un original d'impression sur une plaque flexographique, le procédé comprenant le fiait :
(a) de faire fondre une encre à changement de phase durcissable par rayonnement composée d'au moins un monomère durcissable, d'au moins un gélifiant, d'au moins un photo-initiateur et d'un colorant facultatif,
(b) de déposer l'encre fondue sur la plaque flexographique selon un motif pour former une couche du motif,
(c) de permettre à la couche déposée de l'encre de se gélifier sur la plaque flexographique,
(d) de déposer l'encre fondue sur la couche déposée précédente pour former une couche supplémentaire,
(e) de permettre à la couche déposée supplémentaire de se gélifier,
(f) de répéter les étapes (d) à (e) afin de former d'autres couches déposées et gélifiées supplémentaires, jusqu'à ce que l'original d'impression avec une épaisseur suffisante soit formé sur la plaque flexographique, et
(g) de durcir l'encre sur la plaque flexographique lorsqu'on atteint l'épaisseur suffisante,
(h) où la viscosité de l'encre fondue va de 0,001 à 100 Pa·s (10⁰ cP à 10⁵ cP) à une température allant de 60°C à 100°C.

9. Procédé de la revendication 8, dans lequel l'encre est durcie par l'exposition de l'encre aux rayons ultraviolets.

10. Procédé de la revendication 8 ou 9, dans lequel le dépôt de l'encre pour la couche déposée se produit en un seul passage d'un dispositif d'impression.

11. Procédé de l'une des revendications 8 à 10, dans lequel le dépôt de l'encre pour la couche déposée supplémentaire et l'autre couche déposée supplémentaire se produit en un seul passage d'un dispositif d'impression.

12. Procédé de l'une des revendications 8 à 11, dans lequel une épaisseur totale de la couche déposée, de la couche déposée supplémentaire et des autres couches déposées supplémentaires va de 0,01 mm à 100 mm.

13. Procédé de l'une des revendications 8 à 12, dans lequel l'encre fondue est déposée par jet de l'encre fondue à partir d'un dispositif d'impression en une seule fois afin de former la couche déposée et la couche déposée supplémentaire.

14. Procédé de formation d'un original d'impression sur une plaque flexographique, le procédé comprenant le fiait :
(a) de faire fondre une encre à changement de phase durcissable par rayonnement composée d'au moins un monomère durcissable, d'au moins un agent de changement de phase, d'au moins un photo-initiateur et d'un colorant facultatif,
(b) de déposer l'encre fondue sur la plaque flexographique selon un motif afin de former une couche dans le motif,
(c) de permettre à la couche déposée de l'encre de se gélifier sur la plaque flexographique,
(d) de déposer une couche supplémentaire de l'encre fondue sur la couche déposée précédente,
(e) de permettre à la couche déposée supplémentaire de se gélifier,
(f) de répéter les étapes (d) à (e) afin de former d'autres couches déposées et gélifiées supplémentaires, jusqu'à ce que l'original d'impression avec une épaisseur initiale soit formé sur la plaque flexographique,
(g) de durcir l'encre sur la plaque flexographique afin de former une partie initiale de l'original d'impression,
(h) de déposer une couche de durcissement post-initiale de l'encre fondue sur la partie initiale de l'original d'impression,
(i) de permettre à la couche de durcissement post-initiale déposée de l'encre fondue de se gélifier sur la plaque flexographique,
(j) de déposer une couche de durcissement post-initiale supplémentaire de l'encre fondue sur la couche de durcissement post-initiale déposée précédente,
(k) de permettre à la couche de durcissement post-initiale déposée supplémentaire de se gélifier,
(l) de répéter les étapes (j) à (k) afin de former d'autres couches déposées et gélifiées supplémentaires de durcissement post-initiales, jusqu'à ce que l'original d'impression avec une épaisseur suffisante soit formé sur la plaque flexographique, et
(m) de durcir l'encre sur la plaque flexographique lorsqu'on atteint l'épaisseur suffisante.

15. Procédé de la revendication 14, dans lequel l'épaisseur initiale de l'original d'impression va de 5 à 60 pourcent de l'épaisseur suffisante.
